

July 28, 1942.

W. WHITEHEAD

2,290,929

PRODUCTION OF ARTIFICIAL FILAMENTS

Filed March 20, 1940

Fig. 1.



Fig. 2.



INVENTOR

William Whitehead

BY

Walter & Weir

ATTORNEYS

## UNITED STATES PATENT OFFICE

2,290,929

## PRODUCTION OF ARTIFICIAL FILAMENTS

William Whitehead, Rye, N. Y., assignor to  
Celanese Corporation of America, a corpora-  
tion of Delaware

Application March 20, 1940, Serial No. 324,965

4 Claims. (Cl. 18—54)

This invention relates to the manufacture of artificial or synthetic filaments, and relates more particularly to a novel method of an apparatus for the manufacture of artificial or synthetic filaments of improved textile characteristics.

In the manufacture of artificial or synthetic filaments from solutions of cellulose derivatives in volatile solvents by methods in which the solutions are extruded into a setting medium, the extruded filaments, either singly or associated together as threads, are led, with or without twisting, to bobbins or other winding supports or devices, located outside of the spinning cabinet on which they are wound. Heretofore the thread of associated filaments was led through a guide positioned substantially at the opening leading from the spinning cabinet, passed through said opening, wound about a feed or godet roller and finally wound on to a bobbin or like support, the feed or godet roller operating at such a speed that the filaments were drawn down or extended more or less to produce filaments of increased strength and of the denier desired.

I have now found that cellulose derivative filaments of highly desirable characteristics may be obtained by extruding the cellulose derivative spinning solution into the form of filaments and then collecting them without drawing them down. In accordance with my process, the extruded filaments are permitted to fall of their own weight whereby they are allowed to contract in length. The denier of the filaments formed by my novel process will vary with the length of the cabinet or the length of the fall of the filaments. Thus, where the formed filaments fall through a greater distance the filaments have a greater unsupported length and the weight thereof tends to stretch the same. Accordingly, filaments of the finer denier result. Furthermore, the denier of the filaments formed may be varied by varying the size of the orifices in the spinning nozzle.

Filaments produced in accordance with my invention have been found to have increased strength and an elongation from 40 to 50% greater than filaments produced by prior methods, greater resiliency and greater thermal insulating properties. Moreover, the filaments produced according to my novel process have a rougher surface longitudinally thereof than filaments made by prior processes, i. e. they have a plurality of continuous or irregular relatively deep indentations or canals extending along the length thereof. Such rough surface filaments

are particularly suitable for the production of staple fiber since they have natural, inherent good spinning qualities and substantially permanent binding power, thereby obviating the necessity of putting a crimp in the same. Blankets, suitings and like fabrics made from such staple fibers are substantially free from shedding and have higher thermal insulating qualities presumably on account of the air spaces between the 10 deep striations in the filaments.

It is an important object of this invention to provide a process for the economic and expeditious manufacture of artificially produced filaments having increased strength and elongation, 15 greater resiliency and greater thermal properties than artificial filaments heretofore made.

Another object of this invention is the production of staple fibers of improved textile characteristics.

20 A further object of this invention is the provision of a simple, efficient and inexpensive apparatus for producing the improved filaments.

Other objects of this invention will appear from the following detailed description.

25 In the accompanying drawing, wherein one embodiment of my invention is shown,

Fig. 1 is a diagrammatic representation of a portion of a metier with means for withdrawing the filaments therefrom, and

30 Fig. 2 is a detailed view showing the filaments being led to a device for converting the same into staple fiber.

Like reference numerals indicate like parts in both views of the drawing.

35 Referring now to the drawing, the metier, which is generally indicated by reference numeral 3, may contain any desired number of spinning nozzles 4 arranged in the upper part of the metier, each being formed with a number of spinning orifices to form a corresponding number of filaments. While Fig. 1 shows a metier having five compartments or cells 5 separated from each other by vertical partitions 6 and each containing one spinning nozzle, it is to be understood that any suitable number of such compartments or cells may be arranged in a row and that each of said compartments or cells have more than one spinning nozzle.

40 The spinning nozzles are, of course, supplied with the spinning solution from any convenient supply header, not shown, and the metier is insulated in any suitable manner as is well known in the art.

45 The filaments 1 as they are formed are permitted to fall of their own weight upon an endless conveyor belt 8, carried by pulleys 9 and 11

driven in any suitable manner, which conveyor belt removes the filaments from the meter. Since no tension is applied to the filaments they contract in length before meeting the conveyor belt 8. Preferably, the conveyor belt is arranged to travel at a linear speed equal to or less than the rate of speed at which the filaments fall. The lower edges of the walls of casing 3 should be as close as possible to the conveyor belt 8 or otherwise so arranged as to admit little external air.

A roller 12, which may be an idler and of any suitable size, is positioned above the pulley 11 and with the conveyor belt 8 acts as a nip roller arrangement through which the collected filaments pass and are fed forward. Suitably spaced from the pulley 11 and the roller 12 are nip rollers 13 and 14 which preferably rotate at a peripheral speed greater than that of the roller 12 and the conveyor belt 8, whereby the filaments in the sliver 15 are caused to straighten out.

The nip rollers 13 and 14 feed the sliver into a coiling can 16. Or the sliver may be wound upon a support by any suitable winding device. However, as shown in Fig. 2, a sliver 15 may be passed from the conveyor belt 8 towards a cutting device, generally indicated by reference 17, by the agency of an ejector device generally indicated by reference numeral 18, the sliver passing through the cone 19 of the ejector device and a blast of compressed air or other fluid admitted from the conduit 20 to annular space 21, which blast of compressed air draws or sucks the filaments of the sliver through the apex of the cone carrying the sliver to the cutting devices.

The cutting device comprises a rotating member 22 mounted on a rotating shaft 23 and has any suitable number of plates or knives 24. These blades or knives cooperate with a stationary blade 25 mounted on a block 26 which may be adjustable with respect to the rotating blades 24 by means of a screw bolt 27. The cut staple made up is blown into a chute 28 and collected in a suitable receptacle not shown. If it is desired to apply a finish to the filaments, it is preferable to apply the same while the filaments are still on the conveyor belt.

My invention is particularly applicable to the production of artificial filaments or staple fibers having a basis of cellulose acetate or other cellulose derivative produced by the dry or evaporative method of spinning. Examples of other cellulose derivatives which may form the basis of the filaments or staple fibers are cellulose propionate, cellulose butyrate, cellulose aceto-propionate, cellulose aceto-butyrate, thiocarbamic and alkoxy alkacetyl esters of cellulose, cellulose ethers such as ethyl and benzyl cellulose, and the condensation products of cellulose with glycols or other polyhydric alcohols. Similarly ester-ethers

of cellulose such as, for example, acetates of cellulose hydroxy ethyl-ethers may be employed.

It is to be understood that the foregoing detailed description is merely given by way of illustration and that many variations may be made therein without departing from the spirit of my invention.

Having described my invention, what I desire to secure by Letters Patent is:

10 1. Process for the production of artificial filaments or threads, which comprises extruding in a downward direction a spinning solution into a setting medium, permitting the formed filaments to fall of their own weight, without the application thereto of extraneous tension, on to a conveying surface moving at substantially the same rate of speed as the speed at which the formed filaments fall on to said surface and transporting the filaments on said surface from beneath the point at which they are extruded.

15 2. Process for the production of artificial filaments or threads, which comprises extruding in a downward direction a spinning solution containing cellulose acetate and a volatile solvent therefor into an evaporative atmosphere, permitting the formed filaments to fall of their own weight, without the application thereto of extraneous tension, on to a conveying surface moving at substantially the same rate of speed as the speed at which the formed filaments fall on to said surface and transporting the filaments on said surface from beneath the point at which they are extruded.

20 3. Process for the production of artificial filaments or threads, which comprises extruding in a downward direction a spinning solution into a setting medium and permitting the formed filaments to fall of their own weight, without the application thereto of extraneous tension, on to a conveying surface moving at substantially the same rate of speed as the speed at which the formed filaments fall on to said surface, collecting the filaments from said surface in the form of a sliver and applying a tension on said sliver to straighten the filaments thereof.

25 4. Process for the production of artificial filaments or threads, which comprises extruding in a downward direction a spinning solution containing cellulose acetate and a volatile solvent therefor into an evaporative atmosphere and permitting the formed filaments to fall of their own weight, without the application thereto of extraneous tension, on to a conveying surface moving at substantially the same rate of speed as the speed at which the formed filaments fall on to said surface, collecting the filaments from said surface in the form of a sliver and applying a tension on said sliver to straighten the filaments thereof.

45 WILLIAM WHITEHEAD.